

## UNITED STATES PATENT OFFICE

2,363,515

## HYDROCARBON OILS

Bruce B. Farrington and James O. Clayton,  
Berkeley, and Dorr H. Etzler, Albany, Calif., as-  
signors to Standard Oil Company of California,  
San Francisco, Calif., a corporation of Dela-  
ware

No Drawing. Application December 3, 1942,  
Serial No. 467,779

## 21 Claims. (Cl. 252—53)

This invention relates to new and useful compositions of matter and to methods of preparing the same. In particular, it relates to compositions comprising hydrocarbons of the lubricating oil class, in major part, in which are dissolved or suspended minor amounts of certain metal salts of organic aliphatic carboxylic acids, either alone or in admixture with other compounding agents of the same or different type.

This application is a continuation-in-part of our copending application Serial No. 322,946, filed March 8, 1940, now Patent No. 2,349,817.

It has long been the desire of the lubricating oil compounding art to obtain an oil, particularly of petroleum origin, which alone or with the addition of relatively small amounts of compounding agents, would resist deterioration or degradation when subjected for long periods of time to high temperatures and pressures, in the presence of metals, air or oxygen, or hydrocarbon partial combustion products. Deterioration of the character referred to here manifests itself in diverse effects, dependent upon the nature and degree of refinement of the hydrocarbon oil and upon the environment to which it is subjected, but reference may be made to Diesel engine piston ring sticking, in which the exposure of a lubricating oil to such temperatures as 425°—650° F., in the presence of oxidizing combustion gases at pressures as high as 750—1150 lbs./sq. in., causes the deposition of oil degradation products of such a cementitious character as to effectively take piston rings out of service; to the deposition of "sludge" from automobile crankcase oils, apparently as the result of oxidation and/or polymerization phenomena; and to the corrosion of metal bearing surfaces, apparently as a result of phenomena which cause the formation of organic acidic products. This situation is aggravated by the fact that improvements in the mechanical arts have brought about increasing severity in the conditions to which hydrocarbon oils are subjected, and by the fact that oil compounding designed to effect a stability in one direction often brings about a marked instability in another.

It has been found that the addition to a lubricating oil of small amounts of a metal salt of an aliphatic carboxylic acid, carrying a substituted or unsubstituted carboxylic acid group in addition to the salt-forming carboxylic acid group and carrying in addition to said groups an ether substituent or a keto substituent, or a sulfur, selenium or tellurium analogue of said ether substituent or keto substituent, attached

to an aliphatic carbon atom, brings about an improved stability in hydrocarbon oils when the same are subjected to high temperatures or pressures in the presence of oxygen and metals; such acids correspond in general to the type  $\text{HOOC}-(\text{CH}_2)_n-\text{COOH}$ , in which  $n$  is a whole number; in which there may or may not be alkyl, aryl, aralkyl or aliphatic carbocyclic substitution to increase oil solubility; and in which a polar group selected from the class consisting of  $-\text{OR}_1$ ,  $-\text{SR}_1$ ,  $-\text{SeR}_1$ ,  $-\text{TeR}_1$ ,  $=\text{O}$ ,  $=\text{S}$ ,  $=\text{Se}$  and  $=\text{Te}$  is substituted in a position alpha, beta, gamma, delta or even epsilon to the carbon atom of a salt-forming carboxylic acid group, the effectiveness for the desired purpose decreasing in the order of positions as recited. In the above class of groups  $-\text{OR}_1$ ,  $-\text{SR}_1$ , etc.,  $\text{R}_1$  represents an organic group of essentially hydrocarbon structure such as alkyl, aryl, alkaryl, aralkyl and aliphatic carbocyclic groups. Preferably at least one of said groups is located not more than three carbon atoms from a salt-forming carboxyl group.

Viewed from another standpoint, the salts of this invention are metal salts of polar substituted polycarboxylic acids capable of representation by the partial formula—



in which  $\text{M}$  is a metal, including the hydrogen equivalent of a polyvalent metal,  $\text{R}$  is hydrogen, a metal, ammonium, or an organic group, the groups  $\text{COOM}$  and  $\text{ROOC}$  are attached to aliphatic carbon atoms, the carbon atom to which  $\text{X}$  is attached is an aliphatic carbon atom, preferably alpha, beta or gamma with respect to the  $\text{COOM}$  group, and  $\text{X}$  is selected from the group consisting of  $-\text{OR}_1$ ,  $-\text{SR}_1$ ,  $-\text{SeR}_1$ ,  $-\text{TeR}_1$ ,  $=\text{O}$ ,  $=\text{S}$ ,  $=\text{Se}$  and  $=\text{Te}$ , wherein  $\text{R}_1$  is as defined above, examples of  $\text{R}_1$  being the methyl, ethyl, butyl, hexyl, decyl, tetradecyl, cetyl, phenyl, naphthyl, amylphenyl, cetylphenyl, benzyl and cyclohexyl groups.

The metals whose substituted carboxylic acid salts are useful for the purposes of the invention may have valences from one to four, inclusive, and the salts of potassium, calcium, magnesium, aluminum, chromium, cobalt, lead, manganese, tin and zinc have been found of particular utility.

Among the aliphatic polycarboxylic acids which may be substituted by one or more of the groups  $-\text{OH}$ ,  $-\text{SR}_1$ ,  $-\text{SeR}_1$ ,  $-\text{TeR}_1$ ,  $=\text{O}$ ,  $=\text{S}$ ,  $=\text{Se}$

and  $=\text{Te}$  and used in the form of their metal salts there may be mentioned malonic, succinic, glutaric, adipic and sebatic acids; the alkyl and alkylene homologues of these acids, such as pentylmalonic, cetylmalonic, isopropylsuccinic, centensylsuccinic, and eicosenylsuccinic acids; and various polar substituted (including unsaturated) acids of the same series, such as malic, maleic, tartaric and citric acids.

There are given below the structural formulae of a few typical salts of this invention:

(1) Calcium alpha-cetoxymalonate



(2) Calcium cetyl alpha-methoxymalonate



(3) Calcium cetyl ketomalonate (calcium cetyl mesoxalate)



(4) Calcium alpha-cetoxylsuccinate



(5) Calcium cetyl alpha-methoxy-succinate



(6) Calcium cetyl keto-succinate



(7) Calcium alpha-cetylthiomalonate

(8) Calcium alpha cetyl selenylmalonate

(9) Calcium alpha cetyl tellurylmalonate

(10) Calcium cetylthionomalonate

(11) Calcium cetyl selenomalonate

(12) Calcium cetyl telluromalonate

(13) Calcium cetyl alpha-methylthiosuccinate

(14) Calcium cetyl alpha-methylselenylsuccinate

(15) Calcium cetyl alpha-methyltellurylsuccinate

ate

Compounds 7, 8 and 9 are the thio, seleno and telluro analogues of compound 1, wherein the oxygen of the cetoxy group is replaced by sulfur, selenium and tellurium, respectively. Compounds 10, 11 and 12 are similarly the sulfur, selenium and tellurium analogues of compound 3, and compounds 13, 14 and 15 are the sulfur, selenium and tellurium analogues of compound 5.

The ether substituted malonic and succinic acids and the sulfur, selenium and tellurium analogues of these ether substituted acids (S, Se and Te substituted for O in the group  $\text{OR}_1$ ) can be prepared by well known methods. For instance, alkoxy malonates can be prepared by the method of Wislicenus and Münzschneider (Berichte 1898 vol. 31, p. 552) by condensing alkoxy acetate esters with oxalate esters in dry ether in the presence of sodium followed by a carbon monoxide cleavage to yield the alkoxy malonate esters. The esters can be saponified to yield the acids.

The dialkoxy- and diaryloxy-malonic acids can be prepared by treating dibromomalonate esters with alcoholic solutions of sodium alkoxides or sodium phenates.

The alkoxy succinic acids can be prepared by reacting maleate or fumarate esters with the appropriate alcohol in the presence of a small amount of the sodium alcoholate. This process yields the ester which can be saponified to yield the acid.

The alkylthiosuccinic acids can be prepared by reacting bromosuccinic acid salts with an alkali mercaptide.

The keto, thiono, seleno and telluro malonic and succinic acids can be prepared by well known methods. For instance, salts of ketomalic acid can be prepared by oxidizing malonate esters with nitrogen tetroxide to form the mesoxalate ester (ketomalic) followed by a partial saponification to yield the half ester. Salts of ketosuccinic acids can be prepared by condensing oxalate and acetate esters in the presence of sodium alcoholates in anhydrous ether to form the corresponding ester which can be partially saponified.

From the various acids prepared as described above, the normal and acid salts and the salts of partial esters can be readily prepared by methods well known in the art.

As exemplified by the above structural formulae, the salts of the present invention preferably have in their molecules an oil-solubilizing group, illustrated above by the cetyl group. Other oil-solubilizing groups, such as other alkyl groups, aryl groups, alkyl aryl groups, aryl alkyl groups and cycloaliphatic groups may also be employed. Also, other polar groups may be present in the salt molecule in addition to the indicated ether, keto, and the like groups.

40. Illustrative examples of compositions of the invention are as follows:

1. 99% SAE 30 paraffinic oil  $+1\%$  Ca  $\alpha$ -cetoxy malonate
2. Ditto  $+1\%$  Zn  $\alpha$ -diamylphenoxy malonate
3. Ditto  $+1\%$  Ca  $\alpha$ -cetylthiomalonate
4. Ditto  $+1\%$  Ca cetyl  $\alpha$ -methoxy succinate
5. Ditto  $+1\%$  Ba cetyl  $\alpha$ -methylthiosuccinate
6. 99% SAE 30 naphthenic oil  $+1\%$  Ca laurylmesoxalate
7. Ditto  $+1\%$  Mg dodecyl  $\alpha$ -thionosuccinate
8. Ditto  $+1\%$  Ba cetyl  $\alpha$ -methylselenylsuccinate
9. 99% SAE 30 mixed base oil  $+1\%$  Ca  $\alpha$ -cetoxy malonate
10. Ditto  $+1\%$  Zn  $\alpha$ -diamylphenoxy malonate
11. Ditto  $+1\%$  Ca  $\alpha$ -cetylthiomalonate
12. Ditto  $+1\%$  Ba cetyl  $\alpha$ -methylselenylsuccinate
13. 98% SAE 30 naphthenic oil  $+1\%$  Ca  $\alpha$ -cetoxy malonate  $+1\%$  Ca cetylphenate
14. Ditto  $+1\%$  Ca  $\alpha$ -cetylthiomalonate
15. Ditto  $+1\%$  Ba cetyl  $\alpha$ -methylthiosuccinate
16. Ditto  $+1\%$  Ca cetylphenol sulfonate
17. Ditto  $+1\%$  Mg dodecyl  $\alpha$ -thionosuccinate
18. Ditto  $+1\%$  dicetyl sulfide
19. Ditto  $+1\%$  Ca lauryl mesoxalate
20. Ditto  $+1\%$  dihydroxy diphenyl sulfide

60. These and other oils have been found to be highly useful; among other things they exhibit an enhanced stability toward air at high temperatures and pressures, or less tendency to cause piston ring sticking, or reduced corrosion of bearings of the type of cadmium-silver and copper-lead bearings, or a combination of such valuable properties.

Generally, measurable improvements in the properties of hydrocarbon oils are obtained by the incorporation of as little as 0.1% of the agents of the invention, but amounts between about 0.2% and 2.0% of the agents, by weight based on the oil, are preferable, dependent upon the degree of inherent tendency toward degradation of the oil itself or as otherwise compounded;

amounts higher than about 5.0% are regarded as unnecessary in the best practice of the invention.

A feature of the invention is in the preparation and distribution of bases or concentrates containing relatively large proportions of the additive agents in admixture with hydrocarbon oils of the lubricating or less viscous types or, if more suitable in conjunction with certain other agents, by reason of solubility relationships or the like, in admixture with aromatic hydrocarbons or with alcohols, esters, ketones or ethers, generally of the aliphatic series. Admixtures of the agents and lubricating oils or other solvents or carriers containing upward of 50% of the essential agents, by weight may be thus prepared and distributed, for later blending with the particular lubricating oil media desired to be put to use, as occasion demands. In the preparation of either the finished oils of the invention or the bases or concentrates referred to, complete or clear and homogeneous solution is not always necessary; blending agents or homogenizers may be employed if desirable, to prevent sedimentation of the more oil-insoluble of the agents, but it has been found the possible detrimental effect of the presence of filterable insoluble materials of this character, if indeed present, is determined largely by the particular conditions attending the contemplated use, and that their presence is not in all cases deleterious to the functioning of the compositions in their intended manner.

Herein and in the claims, wherever the term "ether" or "keto" is used to identify a substituent, group or radical, it is intended to identify the group  $-\text{OR}_1$  or  $=\text{O}$ , respectively, wherein the free oxygen valency or valencies are attached to an aliphatic carbon atom other than that of a carboxyl group and wherein  $\text{R}_1$  is as defined above. The sulfur, selenium and tellurium analogues of these substituents, as referred to herein and in the claims, constitute the two classes of substituents: (1)  $-\text{SR}_1$ ,  $\text{SeR}_1$ , and  $-\text{TeR}_1$ , and (2)  $=\text{S}$ ,  $=\text{Se}$  and  $=\text{Te}$ , respectively, in which sulfur, selenium or tellurium take the place of oxygen in the ether ( $-\text{OR}_1$ ) and keto ( $=\text{O}$ ) groups and  $\text{R}_1$  is as defined above.

While the character of the invention has been given in detail and numerous illustrative examples of the preparation and utility of the compositions of the invention have been described, this has been done largely by way of illustration and with the intention that no limitation should be imposed upon the invention thereby. It will be obvious to those skilled in the art that numerous modifications and variations of the above illustrative examples may be effected in the practice of the invention, which is intended to be of the scope of the appended claims.

We claim:

1. A liquid hydrocarbon oil of the lubricating class, normally tending to deteriorate at operating temperatures encountered in the lubrication of internal combustion engines, containing a small amount, sufficient to retard the said deterioration, of a metal salt of an aliphatic polycarboxylic acid substituted on an aliphatic carbon atom not more than about three carbon atoms removed from a salt-forming carboxyl group by a substituent selected from the class consisting of ether and keto substituents and the sulfur, selenium and tellurium analogues of said ether and keto substituents.

2. The oil of claim 1, wherein said substituent is an ether group.

3. The oil of claim 1, wherein said substituent is a keto substituent.

5 4. A liquid hydrocarbon oil of the lubricating class, normally tending to deteriorate at operating temperatures encountered in the lubrication of internal combustion engines, containing a small amount, sufficient to retard the said deterioration, of a polyvalent metal salt of an aliphatic polycarboxylic acid substituted on an aliphatic carbon atom not more than about three carbon atoms removed from a salt-forming carboxyl group by a substituent represented by the formula  $-\text{SR}_1$ , wherein  $\text{R}_1$  is a radical selected from the group consisting of alkyl, cycloaliphatic, aryl, aralkyl and alkaryl radicals.

10 5. A liquid hydrocarbon oil of the lubricating class, normally tending to deteriorate at operating temperatures encountered in the lubrication of internal combustion engines, containing a small amount, sufficient to retard the said deterioration, of a polyvalent metal salt of an aliphatic dicarboxylic acid, said acid containing an oil-solubilizing substituent and being substituted on an aliphatic carbon atom not more than about three carbon atoms removed from a salt-forming carboxyl group by a substituent selected from the class consisting of ether and keto substituents

15 30 and the sulfur, selenium and tellurium analogues of said ether and keto substituents.

35 6. A liquid hydrocarbon oil of the lubricating class, normally tending to deteriorate at operating temperatures encountered in the lubrication of internal combustion engines, containing a small amount, sufficient to retard the said deterioration, of a polyvalent metal salt of an aliphatic tricarboxylic acid, said acid containing an oil-solubilizing substituent and being substituted on an aliphatic carbon atom not more than about three carbon atoms removed from a salt-forming carboxyl group by a substituent selected from the class consisting of ether and keto substituents and the sulfur, selenium and tellurium analogues of said ether and keto substituents.

40 7. A composition of matter, comprising a major proportion of a hydrocarbon oil of lubricating viscosity and a small amount, sufficient to retard the deterioration of the oil, of a compound represented by the partial formula



55 55 wherein M is a metal, the group  $\text{COOR}$  is selected from the class consisting of free carboxyl, salt-forming carboxyl and carboxy ester groups, both  $\text{COOR}$  and  $\text{COOM}$  are attached to aliphatic carbon atoms, the carbon atom to which X is attached is an aliphatic carbon atom, and X is selected from the group consisting of ether and keto substituents and the sulfur, selenium and tellurium analogues of said ether and keto substituents.

60 60 8. A composition of matter, comprising a major proportion of hydrocarbon oil of lubricating viscosity and about 0.1 to 5 per cent by weight based on finished oil of a compound of the structure



65 70 wherein M is the hydrogen equivalent of a polyvalent metal,  $\text{COOR}$  is selected from the class

75 consisting of free carboxyl, salt-forming carboxyl

and carboxy ester groups, both COOR and COOM are attached to aliphatic carbon, X is attached to aliphatic carbon, and X is selected from the group consisting of ether and keto substituents and the sulfur, selenium and tellurium analogues of said ether and keto substituents, said compound also containing an oil-solubilizing group.

9. The composition of claim 8, wherein X is an ether group.

10. The composition of claim 8, wherein X is the sulfur analogue of an ether group.

11. The composition of claim 8, wherein X is a keto substituent.

12. The composition of claim 8, wherein X is selected from the class consisting of -OR<sub>1</sub>, -SR<sub>1</sub>, -SeR<sub>1</sub> and -TeR<sub>1</sub>, wherein R<sub>1</sub> is a high molecular weight, oil-solubilizing ether-forming organic group.

13. A petroleum lubricating oil containing about 0.1 to 5 per cent by weight based on finished oil of a polyvalent metal salt of an alkoxy substituted malonic acid, the alkyl group of the alkoxy substituent being a higher alkyl group capable of imparting oil-solubility to the salt.

14. The composition of claim 13, wherein said polyvalent metal is an alkaline earth metal.

15. The composition of claim 13, wherein said polyvalent metal is calcium.

16. A petroleum lubricating oil containing about 0.1 to 5 per cent by weight based on finished oil of a compound of the structure



wherein M is a polyvalent metal and R<sub>1</sub> and R<sub>2</sub> represent the same or different high molecular weight oil-solubilizing organic radicals.

17. A petroleum lubricating oil containing 40

about 0.1 to 5 per cent by weight based on finished oil of a polyvalent metal salt of an alkoxy substituted succinic acid, the alkyl group of the alkyl ether substituent being a higher alkyl group capable of imparting oil solubility to the salt.

18. The composition of claim 17, wherein said polyvalent metal is an alkaline earth metal.

19. A petroleum lubricating oil containing about 0.1 to 5 per cent by weight based on finished oil of a polyvalent metal salt of a partial ester of a keto substituted succinic acid, the ester group of said partial ester containing a high molecular weight oil-solubilizing organic radical.

20. A concentrated dispersion in mineral oil of a metal salt of an aliphatic polycarboxylic acid substituted on an aliphatic carbon atom not more than about three carbon atoms removed from a salt-forming carboxyl group by a substituent selected from the class consisting of ether and keto substituents and the sulfur, selenium and tellurium analogues of said ether and keto substituents.

21. A petroleum lubricating oil tending normally to deteriorate and form carbonaceous deposits on pistons when used as the crankcase lubricant of an internal combustion engine and a small amount each, sufficient to retard said deterioration and deposition, of a polyvalent metal salt of an alkylated phenol and a polyvalent metal salt of an aliphatic polycarboxylic acid substituted in a position not more than about three carbon atoms removed from a salt-forming carboxyl group by a substituent selected from the class consisting of ether and keto substituents and the sulfur, selenium and tellurium analogues of said ether and keto substituents.

BRUCE B. FARRINGTON.

JAMES O. CLAYTON.

DORR H. ETZLER.